

Sept. 19, 1944.

T. F. BANIGAN ET AL

2,358,376

PROCESS FOR THE MANUFACTURE OF REGENERATED CELLULOSE RIBBONS

Filed Nov. 1, 1941



Fig. 2



Fig. 3

Thomas F. Banigan  
Ray E. Hartman INVENTOR.

Fig. 1

BY  
Paul B. Miller  
ATTORNEY

## UNITED STATES PATENT OFFICE

2,358,376

PROCESS FOR THE MANUFACTURE OF  
REGENERATED CELLULOSE RIBBONS

Thomas F. Banigan, Kenmore, and Roy E. Hartman, Buffalo, N. Y., assignors to E. I. du Pont de Nemours & Company, Wilmington, Del., a corporation of Delaware

Application November 1, 1941, Serial No. 417,581

2 Claims. (Cl. 18—47.5)

This invention relates to a process of manufacturing shrinkable, non-fibrous, secondary closure devices, especially regenerated cellulose and like ribbons adapted upon shrinking to tightly fit over and satisfactorily seal the primary closure to a bottle, or the like.

Shrinkable, non-fibrous, secondary closure bands for bottles have been known and used for years. They provide an attractive decoration to the container, a deterrent against tampering with the contents thereof, and facilitate compliance with the law which requires that a part of the government revenue stamp remain on the bottle of alcoholic beverages until the contents have been dispensed. An extensively used type of band is that having opaque and clear sections. The opaque sections, being suitably pigmented, provide an attractive background for printed matter (advertising, directions for opening, etc.), and the clear sections, when suitably positioned, permit observation of the revenue stamp without removal of the secondary closure. U. S. A. Patents 1,647,489 (Webster), 2,121,042 (Morgan) and 2,161,561 (Dalton) are representative of the art treated in the foregoing résumé. The conventional details of band manufacture are disclosed in the foregoing U. S. A. patents and 2,141,776 (Vautier & Fays), and since the processing of these articles is analogous to that employed with cellulosic sheet (see U. S. A. Patents 1,548,864, 1,601,289 and 2,123,883), reference is made to such prior art in the interest of brevity.

For some time an insistent and appreciable demand for a ribbon or tape secondary closure, to be used instead of the closed band or tube section, has existed. Inasmuch as the extent of this demand and the possibilities of the development are still somewhat indeterminate, it would be very advantageous if some means for preparing such ribbons with existing apparatus could be discovered for use at least until evaluation of the market has become possible.

When continuous lengths of regenerated cellulose sheet are prepared in the conventional manner, the edges are quite irregular, and there is an undesirable thickening of the marginal portion. It is necessary to remove this thickened bead and adjacent portion of the film in order to provide a regular edge on the material to be offered to the trade. This wastage is not an insurmountable difficulty when wide sheets (four or five feet in width) are being manufactured, because of the percentage or relative proportion of the scrap to the good material, but in a

narrow tape (a few inches in width) the percentage of loss militates against such a type of manufacture.

If a means for preparing sheet material without the formation of the irregular edge and bead could be discovered, it also would greatly advance the art.

The primary object of this invention was to overcome the aforementioned and other difficulties encountered in the preparation of ribbon secondary closures. Other objects will appear hereinafter.

It has now been found that existing apparatus can be used, beaded and irregular edge formation avoided, and a very satisfactory ribbon secondary material produced, by extruding viscose in the manner heretofore employed in the preparation of regenerated cellulose tube, and slitting the tube after coagulation and during regeneration but before the conventional purifying processing takes place.

How the foregoing objects and related ends are accomplished will be apparent from the following exposition, in which are disclosed the principle and divers embodiments of the invention, including the best mode contemplated for carrying out the same. Parts are given by weight throughout the specification unless otherwise specified. The written description is amplified by the accompanying drawing, in which:

Figure 1 is a diagrammatic side elevation view, partly in section, with some of the parts exaggerated in the interest of clarity, of the tube slitting arrangement of the present invention;

Figure 2 is an elevation view corresponding to the upper part of Figure 1, taken at right angles to the view of Figure 1; and

Figure 3 is a fragmentary conventionalized perspective view, with parts exaggerated for clearness, of the cutting device.

*Example*

A cellulosic tube having 4 longitudinal sections alternately clear and pigmented was prepared by extruding viscose in the manner set out in U. S. A. Patent No. 2,141,776. The viscose contained 7% cellulose and 6% sodium hydroxide. The viscose used in the opaque sections contained, in addition, 1% titanium dioxide (based on the weight of the viscose). The viscose was extruded upwardly into an aqueous bath containing 15% sulfuric acid and 16% sodium sulfate.

The continuous tubing passed at the rate of approximately 75 feet per minute through 72

inches of this coagulating bath. After emerging from the bath and traveling approximately 2.0 feet, the tube was slit by a cutting device comprising a straight knife blade operating in conjunction with a circular sharpened disc which rotated against the blade. A stream of air directed into the open tubing just above the slitter kept the tube dilated and free from creases.

The slit tube was then passed under a spreader rod and over a roll to open the tube and flatten the resulting web, after which it was passed into a regenerating bath. A negligible amount of regeneration took place before the slitting operation. This situation prevails even when the coagulation bath has a high acid content, because the tubing is not in contact with the coagulating solution for a sufficiently long time to appreciably regenerate the cellulose. In the regeneration bath the time of treatment and strength of acid are correlated to finish the regeneration.

The regenerated band was then conducted through a series of treatment vats for desulfuring, bleaching, etc., in the conventional manner for processing regenerated cellulose. Printing was then applied to the opaque sections in the customary manner (see U. S. A. Patent No. 1,897,769 to Fletcher).

At the time of slitting, the tube had a perimeter of approximately 130 millimeters and a thickness of 0.014 inch. After processing, the web was 104 millimeters wide and had a thickness of 0.010 inch. The finished gel ribbon had no significant thickening or swelling at the margins, and the margins were quite regular. These advantages would also appear if large tubes, for example, those having a circumference of around 50 inches, were similarly processed.

Some of the gel web, produced by this method, was severed immediately into strips, tapes or ribbons by a transverse cut, and stacked while the remainder was rolled into stock rolls. The automatic machinery for applying the strips is of two types. One uses stacked individual strips, and the other a roll of material from which the strips are cut as needed.

A suitable adhesive (for example, an aqueous solution containing 10% polyvinyl alcohol and 5% hydrolyzed gelatin) was applied, and the strips sealed about the necks and primary closures of bottles containing the labels, revenue stamps, etc., and allowed to dry. The adhesive applied at the overlapping portions of the ribbon held the band in place, and the shrinkage resulting from the drying of the gel ribbon caused the secondary closure to conform to the contour of the bottle upon which it was placed. The dried article had good durability and practically uniform physical properties across its width. The transparency of the clear sections was very satisfactory.

The lengthwise slitting of the tube may take place before, during or after regeneration. Because of difficulties in processing tubing satisfactorily, it is preferred to slit the tubing before it passes the first support after leaving the coagulating bath. In this mode of operation the web is formed after the gel body has lost its ability to form a beaded edge, and the process is

therefore not only a satisfactory temporary means of making ribbon seals while the market is crystallizing, but also promises to be suitable for eventual commercial scale production.

5 The invention is not limited to regenerated cellulose, since similar ribbons (or continuous strips) may be prepared from other aqueous or aqueous alkaline solutions or dispersions of cellulosic substances, such as those employed in the cuprammonium regenerated cellulose and aqueous alkali soluble low substituted cellulose ethers (see U. S. A. Patents 2,234,016 to Woodhouse and 2,123,883 to Ellsworth) manufacturing procedures.

10 The products of this invention may be colored in any desired manner, for example, by pigmenting the viscose or dyeing the shaped product. Other types of ornamentation or decoration for such products are well known in the art and may be employed, or if desired, the entire tube and resulting ribbon may be clear and transparent.

15 In order to give uniform tubing, it is desirable that the walls of the extrusion orifice be concentric circles. A slight variation into an elliptical form may be employed so long as the clearance of the two walls is uniform and the eccentricity of the ellipse is not so great as to unduly distort the web when flattened.

20 Various slitting devices may be employed in opening up the tubing. Good results can be obtained with rotary shears, vibrating shears, etc., but the combination knife and disc has been found especially satisfactory.

25 As many apparently widely different embodiments of this invention may be made without departing from the spirit and scope thereof, it is to be understood that this invention is not limited to the specific embodiments thereof except as defined in the appended claims.

30 We claim:

1. In the production of a regenerated cellulose ribbon, the steps comprising continuously extruding viscose in the form of a tube, continuously coagulating the tube in a coagulating bath, continuously withdrawing the coagulated tube from the coagulating bath, dilating the coagulated tube with an air jet as it passes from said coagulating bath, slitting the tube longitudinally 35 while it is dilated by said air jet whereby to form a ribbon, and passing said ribbon into a regenerating bath to complete the regeneration thereof.

40 2. In the production of a regenerated cellulose ribbon, the steps comprising continuously extruding viscose in the form of a tube, continuously coagulating the tube in a coagulating bath, continuously withdrawing the coagulated tube from the coagulating bath, dilating the coagulated tube with an air jet as it passes from said coagulating bath, slitting the tube longitudinally 45 approximately 2 feet from said coagulating bath while it is dilated by said air jet whereby to form a ribbon, and passing said ribbon into a regenerating bath to complete the regeneration thereof.

45 THOMAS F. BANIGAN.  
ROY E. HARTMAN.